

## UNITED STATES PATENT OFFICE

1,995,900

## PRODUCTION OF BAST FIBERS FOR PAPER-MAKING AND OTHER PURPOSES

George A. Richter, Berlin, N. H., assignor to Brown Company, Berlin, N. H., a corporation of Maine

No Drawing. Application December 28, 1932,  
Serial No. 649,154

7 Claims. (Cl. 92—8)

This invention relates to the production of bast fibers or bast fiber pulp for paper-making and other purposes, including the manufacture of yarns and textile fabrics.

There are various vegetable plants like ramie, hemp and flax, which bear so-called bast fibers, that is, fibers which occur as the external or surface layer of the plant stalks and which extend for the entire length of the stalks. The bast fibers are characterized by their excellent physical and chemical qualities, whereas the rest of the fibers are of a comparatively short length and of a distinctly lower order of quality. The object of the present invention is the segregation of the bast fibers in an advantageous condition from the short fibers so that the bast fiber portion may serve for those purposes to which it is best adapted, and the short fiber portion may serve in other connections for which it is most useful.

In accordance with the present invention, stalks of the foregoing character are first cut across their longitudinal axes into chips or cylindrical pieces of a length commensurate with the fiber length desired in the long fiber portion to be segregated and recovered from the mass of mixed fibers into which the stalks can be resolved. The chips are then subjected to the fiber-liberating action of a suitable chemical pulping or cooking liquor, for instance, an alkaline cooking liquor such as is used in the production of so-called kraft or soda pulps or an acid cooking liquor such as is employed in the production of so-called sulphite pulp. The chemical pulp thereby produced consists of a mass of fibers made up of the comparatively long bast fibers and the shorter fibers originating in the internal structure of the stalks. The longer bast fibers are distinguishable chemically from the shorter fibers in that, in the case of ramie, for example, they are of lower pentosan and lignin content than the short fibers. Even when cut to short length as by beating action preparatory to paper-making, the bast fibers show physical distinctions, which are observable under the microscope, from the short fibers derived from the internal structure of the ramie stalk. In accordance with my invention, the bast fiber portion of the chemical pulp is separated practically in entirety from the short fibered portion through the use of suitable apparatus, for instance, apparatus of the type disclosed in U. S. Patent No. 1,786,973, issued December 30, 1930 to Robert A. Webber. Apparatus such as is disclosed in that patent is designed to select and remove the long fibered portion of a pulp through the action of edge-presenting members, e. g., grills, which, as they are moved through a pulp suspension of the appropriate consistency, pick up the long fibers while by-passing the short ones. Such an apparatus is of particular value in selecting or segregating the long bast fiber por-

tion of a pulp liberated from ramie or similar stalks because the bast fibers are distinctly longer than the rest of the pulp and little, if any, bast fiber is missed by the selecting apparatus even when the pulp is passed through the apparatus only once.

Let us assume, for example, that the original stalks are chopped or cut into chips whose length approximate about one-half inch. In some cases, it may be desirable to debark the stalks or chips so as to promote subsequent fiber-liberating action as well as to enhance the cleanliness of the liberated fibers or pulp. The chips can be subjected under fiber-liberating conditions to the action of a kraft cooking liquor which, as is well known, contains caustic soda and sodium sulphide as the fiber-liberating chemicals. If desired, the cooking liquor may be a soda liquor, that is, one containing substantially only caustic soda as the fiber-liberating chemical. An acid cooking liquor such as a sulphurous acid solution of calcium sulphite, sodium sulphite, or the like, may be used to effect the pulping of the stalks. Indeed, any suitable chemical pulping liquor, including a straight solution of sodium sulphite, may be used under conditions to dissolve the encrusting or cementitious content of the stalks, thereby liberating the ultimate fibers of which the stalks are composed. The resulting pulp is washed free of chemical cooking liquor and is put through suitable selecting mechanism which functions to segregate the bast fiber portion, which, in the present example, consists of fibers of substantially one-half inch length, from the rest of the fibers which possess an average fiber length of about one-sixteenth inch. A typical chemical pulping liquor such as a kraft or soda liquor will afford a yield of dry pulp of about 50%, based on the weight of the dry raw stalks. The raw stalks in the case of ramie bear about 10% by weight of bast fiber, the rest of the stalk consisting of the short fibered interior portion, pith, and cementitious material, which latter two constituents are largely dissolved in the chemical pulping liquor.

The separated, long fibered bast portion being of lower ligneous and resin content than the short fibered portion is more easily bleachable to whiteness than the short fibered portion. In the case of stalks which have been pulped in an acid sulphite or similar cooking liquor, the long fibered bast portion needs little, if any, bleaching to become white. In fact, the long fibered bast portion may be used in the condition that it is separated from the pulp mass as a whole, that is, without bleaching, for paper-making and for the manufacture of yarns and textile fabrics. When used for paper-making, the long fibered portion yields papers of high strength, toughness, and other physical characteristics. Such papers are

similar in their characteristics to high grade rag or linen papers as heretofore made. The short fibered portion may, after bleaching or other suitable chemical treatment, serve as a constituent 5 in papers of comparatively low quality, e. g., book or magazine papers, such as heretofore made from comparable short fibered pulps such as soda pulp. Either the long fibered or short fibered portions may be subjected to refinement in alkaline liquors and/or to bleaching treatment, if desired; or the pulp as a whole may undergo such processing before it is classified or graded into its long fibered and short fibered components. It is, however, preferable to treat each fiber portion 10 independently, for, as hereinbefore indicated, the two portions respond differently to chemical treatment and are best adapted for different purposes, which usually require different chemical conditioning treatments for the fiber. 15

20 In some instances, the raw stalks may be exposed to the action of chlorine water, hypochlorite liquors, or similar oxidants, which extract ligneous and other undesirable constituents from the raw stalks or promote their dissolution in the chemical cooking liquor to which the stalks are subsequently subjected.

25

It is of course possible to cause chemical pulping of the whole stalks, but in such case one encounters the difficulty of producing such long bast fibers that they tend to become so badly tangled or knotted as to give rise to difficulty of selection. Again, while tangling or knotting of the bast fibers may not be especially serious in paper-making, which requires the use of the 30 beater engine for reducing the fibers to paper-making condition, tangled or knotted fibers would not lend themselves with facility to textile-making operations performed through the action of carding, combing, and similar machines on the substantially dry fibers. Accordingly, it is distinctly preferable that the stalks be cut into chips of the appropriate length before the chemical pulping operation. When the separated, long fibered bast portion is to serve in textile-making 35 operations, the chips may be of a length of, say 1 to 3 inches, as fibers of such length can be readily carded, combed, spun, twisted, and otherwise treated like cotton fiber. When this portion is to enter into paper-making operations, or is to 40 be formed into rovings or yarns through the furling of damp pulp ribbons produced on machinery of the paper-making type, or through the twisting of paper strips, the chips may be of a length of, say one-half to one inch, that is, of a length 45 distinctly greater than the average fiber length of wood pulp but not unduly long, as otherwise it would be necessary to expend considerable energy in the beater engine in reducing the fibers to satisfactory paper-making length. The fact 50 that the fibers are of a markedly greater length than wood pulp fibers means that even after beating has been effected and the pulp has been hydrated to highly satisfactory paper-making condition, the length of the fibers is such that the 55 papers made therefrom are characterized by their extraordinary toughness, strength, tear resistance, rattle, and other valuable qualities associated with rag and linen papers of the best grade.

I claim:—

70 1. A process which comprises cutting bast fiber-bearing stalks, all of whose fiber is bound up in the stalks, across their longitudinal axes into chips of a length greater than the average fiber length of wood pulp, cooking such chips in

a chemical liquor to liberate the fibers thereof, such fibers consisting of both long bast fibers and short stalk fibers, and selectively removing long bast fibers from the rest of the stalk fibers. 5

2. A process which comprises cutting bast fiber-bearing stalks, all of whose fiber is bound up in the stalks, across their longitudinal axes into chips of a length of at least about one-half inch, cooking such chips in a chemical liquor to liberate the fibers thereof, such fibers consisting of both long bast fibers and short stalk fibers, and selectively removing the bast fibers having a length of at least about one-half inch from the rest of the stalk fibers. 10

3. A process which comprises cutting bast fiber-bearing stalks, all of whose fiber is bound up in the stalks, across their longitudinal axes into chips of a length greater than the average fiber length of wood pulp, cooking such chips in a chemical liquor to liberate the fibers thereof, such fibers consisting of both long bast fibers and short stalk fibers, selectively removing the long bast fibers from the rest of the stalk fibers, beating said removed bast fiber portion, and forming said beaten fiber portion into paper. 15

4. A process which comprises cutting bast fiber-bearing stalks, all of whose fiber is bound up in the stalks, across their longitudinal axes into chips of a length ranging from about one-half inch to about three inches, cooking such chips in a chemical liquor to liberate the fibers thereof, such fibers consisting of both long bast fibers and short stalk fibers, and selectively removing the bast fibers having a length ranging from about one-half inch to about three inches 30 from the rest of the stalk fibers. 35

5. A process which comprises cutting bast fiber-bearing stalks, all of whose fiber is bound up in the stalks, across their longitudinal axes into chips of a length ranging from about one-half inch to about three inches, cooking such chips in a chemical liquor to liberate the fibers thereof, such fibers consisting of both long bast fibers and short stalk fibers, washing the mixed fibers, and selectively removing the bast fibers having a length ranging from about one-half inch to about three inches from the rest of the stalk fibers. 40

6. A process which comprises cutting ramie stalks across their longitudinal axes into chips of a length ranging from about one-half inch to about three inches, cooking such chips in a chemical liquor to liberate all the fibers thereof, such fibers consisting of both the long bast fibers and the short stalk fibers having an average length of only about one-sixteenth inch, and selectively removing the bast fibers having a length ranging from about one-half inch to about three inches from the rest of the stalk fibers. 50

7. A process which comprises cutting ramie stalks across their longitudinal axes into chips of a length ranging from about one-half inch to about three inches, cooking such chips in a chemical liquor to liberate all the fibers thereof, such fibers consisting of both the long bast fibers and the short stalk fibers having an average length of only about one-sixteenth inch, washing the mixed fibers, and selectively removing the bast fibers having a length ranging from about one-half inch to about three inches 65 from the rest of the stalk fibers. 70